

March 3, 1959

R. V. SPENCER

2,875,898

FANNING ORE CONCENTRATOR

Filed Sept. 13, 1954



Inventor  
Robert V. Spencer,  
by George B. Baldwin  
His Attorney.

# United States Patent Office

2,875,898

Patented Mar. 3, 1959

1

2,875,898

## FANNING ORE CONCENTRATOR

Robert V. Spencer, Jacksonville, Fla., assignor to  
James Hall Carpenter, Jacksonville, Fla.

Application September 13, 1954, Serial No. 455,631

13 Claims. (Cl. 209—458)

This invention relates to ore concentrators and particularly to a concentrator embodying a novel fan arrangement for vaning and fanning or spreading and for splitting the stratified stream issuing from the discharge end of a sluice.

A general object of this invention is to improve the concentrating of ores, and more particularly to provide means for spreading and stratifying a stream of granular or comminuted materials entrained in a stream of liquid.

A further object of this invention is to improve the accuracy of splitting of the ore constituents present in a stratified stream of ore particles, and to simplify the appropriate adjustments to splitter members in concentrators.

A still further object of this invention is to provide a pinched sluice type of wet ore concentrator or separator capable of a more complete stratification of ore particles of respectively different sizes, shapes and specific gravities, operative to provide stratification and separation between particles of only slightly different respective specific gravities, sizes and shapes.

Additional general objects of this invention are to provide a sluice separator of greater simplicity capable of handling relatively large amounts of ore in a given time, with high separation or concentration efficiency, at a high pulp density and with minimum water requirements.

It is also an object of this invention to provide a simplified wet feed for a stratifying sluice or trough, which feed will supply a sheet of pulp without surging and with a minimum of discontinuities of pulp density.

Sluice separators, sometimes called concentrators or classifiers, have been in use for a great many years, particularly in connection with the removal of heavy gold particles from relatively light, valueless sand. Spiral concentrators, wet shaking tables and other types of wet gravity concentrators usually occupy considerable space, are of heavy construction and require relatively large quantities of accessory water or "wash water" as an aid in the separation of minerals. The addition of "wash water" along a stream in which stratification is taking place is objectionable not only because of the equipment necessary for its supply but because any interference with the stream is likely to create turbulence in the stream which, in turn, may re-mix the particles which have become stratified or may cause collection of dams built up of particles at the discontinuity in the flow, which dams change the shape of the flow path disadvantageously.

A particular disadvantage of wet type sluice concentrators which have heretofore been suggested lies in the sensitivity of adjustment of stream splitters, and in the necessity of testing the output components to discover the most appropriate setting of the splitters.

Among the objects of the present invention, accord-

2

ingly, are the avoidance of the complexities of other gravity separators and the provision of a simple preconditioning arrangement, such as a simple straight flow sluice of the type having converging sides, the preconditioner having a deep or high and narrow outlet orifice, together with stream vaning and fanning means, and with splitter means capable of ready adjustment, so arranged that the effects of each of several permitted adjustments are clearly and directly seen, permitting the immediate recognition of the need for adjustment without laborious and time-consuming tests of output constituents and the accomplishment of adjustments to the proper setting without trying out several different settings and thereafter awaiting test results to determine the best of the several settings.

15 Certain types of ores, such as those containing titanium minerals, among others, are desirably concentrated by wet gravity concentration means prior to final separation steps performed with electrostatic, magnetic or similar separating machines. The differences in specific gravity between constituents of such ores may be relatively slight and it is an object of this invention to provide means to stratify the constituents with increased accuracy or completeness of stratification, that is, with a minimum of lighter materials in the strata of heavier materials and a minimum of heavier materials in the lighter materials strata. Since lighter materials may be discarded, it is particularly important to avoid the inclusion of substantial quantities of the values in the lighter material strata.

20 It has also been found that titanium ore deposits in certain parts of the world vary markedly within a single deposit as to richness. Thus, while ore delivered from the mine for concentration at one time may comprise only one or two percent heavy minerals, a few minutes later 25 the ore delivered from the mine may have thirty percent heavy minerals. Such variations must be compensated by adjustment of the stream dividing means of the gravity concentrator to prevent excessive losses in the tailings when the ore is rich and to prevent excessive sand in the concentrate output when the ore is less rich.

30 It is, accordingly, a further object of this invention to provide a concentrator permitting ready visual inspection of the stratification of the stream being split and visual determination of the most advantageous splitter settings, together with provisions for rapid readjustment of splitter 35 position to compensate for such variations in richness of ore as soon as the variations are found to occur.

The novel features which are believed to be characteristic of this invention are set forth with particularity in 40 the appended claims. The invention itself, however, both as to its organization and method of operation, together with further objects and advantages thereof, may best be understood by reference to the following description taken in connection with the accompanying drawing, in which:

45 Fig. 1 is a perspective view of a wet ore concentrator in accord with this invention;

50 Figure 2 is a detail back view, in perspective, of the discharge end and fan and splitter portions of the concentrator; and

55 Fig. 3 is a detail end view, in perspective, of the discharge end and fan and splitter portions of the concentrator.

60 A concentrator according to this invention, as shown in Fig. 1, comprises a vertical pulp supply pipe 1 through which the ore pulp is pumped, as by a centrifugal pump, 65 into the lower or apical end of a generally inverted triangular conduit chamber 2. Chamber 2 preferably is of constant thickness, which may be about two inches,

and increases in breadth from about two or three inches at the lower end or apex to about twenty inches at the upper end, and being about twenty-one inches high. The long upper edge at the front of the chamber 2 is formed to provide a lip 3 over which a sheet of pulp flows, while the other three sides of the top of chamber 2 are enclosed with walls terminating sufficiently above the level of the lip to prevent spilling of the pulp except over the lip. The upper end of the conduit 2 may be left open, or closed over as desired.

The sheet of pulp flowing or cascading over lip 3 falls preferably a very short distance and at a very low velocity onto the relatively wide upper end of a downwardly inclined flat bottom portion 4 of a trough or sluice, indicated generally at 5. The sluice 5 may be termed a pinched sluice, in that its upstanding side walls 6 and 7 which confine the flow of pulp gradually approach each other or converge to give a generally triangular shape to the sluice. The side walls 6 and 7 form at their lower or forward ends a tall or high and narrow outlet opening from which the pulp issues in a tall and high stream. During its course down the sluice, the pulp becomes stratified, the heavier materials, that is, the materials of greater specific gravity, dropping in the stream and forming a lower strata, while the lighter materials of less specific gravity tend to remain in the upper portions of the stream and form higher strata. It will be understood that the stratification is not complete, in that the lower portions of the stream contain some percentage of lighter particles and the intermediate and upper strata contain some heavy particles. The usefulness of the concentrator herein disclosed, accordingly, will be primarily to provide from a granular or comminuted ore as mined, and which may comprise a small percentage of, for example, heavy minerals, a concentrate of relatively much higher heavy mineral percentage. In connection with certain specific ores as hereinafter explained it has been found economic and desirable to pass the pulp of ore from the mine through a concentrator according to the invention and to collect a concentrate portion, a middlings portion and a tailings portion from the stream and then to pass the middlings again through the same concentrator, or through another such concentrator. The middlings may, for example, be mixed in with the raw feed for the same unit, or middlings from two units may be passed together into a third unit, and many other variations of the flow plan for re-concentration of middlings will be obvious to those skilled in the art. The tailings may be similarly recirculated in some instances or may be discarded. To permit the separate collection of the three strata as suggested, two splitters in the form of short splitter bars or members are provided for the concentrator shown, although it will be understood that if only one split of the stream into two portions is desired, only one splitter will be required, and, if more than three portions are desired, additional splitters may be employed.

As seen in Fig. 1, splitters or splitter bars 9 and 10 are arranged to extend outwardly from the front face 11 of a vanning and fanning plate member 12, which is preferably flat as shown. Each splitter comprises essentially a wedge-shaped member having a relatively sharp upper cutting edge, such as edge 13, and divergent sides, such as sides 14 and 15. The splitter members shown are formed of sheet metal bent to provide the sharp upper cutting edge 13, downwardly and outwardly inclined sides 14 and 15, and a base portion 16, the base portion of each splitter being affixed by welding or by other suitable means to the end of a respective one of supporting arms 17 and 18.

The splitters 9 and 10 are held firmly against the surface 11 of plate 12 by the supporting arms 17 and 18, and the path of the stream across the plate surface is indicated in broken lines. As the stream courses down the sluice, the stream rises gradually higher on the

walls 6 and 7, and the height of the stream is generally indicated by broken line 19 along wall 6. The stream issues from outlet 8 in the shape outlined between lines 20 and 21 and is intercepted by or impinges upon the plate surface 11 at approximately the area below the break indicated at 22, thereafter fanning out across the plate below and beyond the area of impingement, as indicated by the upward spread of line 23. The stream from the outlet orifice 8 preferably passes freely through the air for about two to four inches before impinging on the plate surface, and the plate surface should be at an average angle of approximately 15 degrees to the direction of the stream as the stream meets the plate, greater angles than about 25 degrees causing undesirably great turbulence on contact and less angles than about 10 degrees yielding less vanning and fanning effect. Since lower parts of the stream may be moving more nearly vertically downwardly than upper parts upon impingement, there is no one angle of impingement, and the impingement angle herein given is therefore as closely as possible approximated as the average angle taking all parts of the impinging stream. A specific setting of the plate position which has proved appropriate, for example, in the specific concentration of ore from Gambia as hereinafter reported comprised a tilting of the plate at an angle of 28 degrees from a line through the plate which line was constructed as perpendicular to the plane of the bottom 4 of the sluice, and the plate was arranged to form an angle of 5 degrees with the center line of the bottom 4 of the sluice, as measured in the plane of the bottom.

The fanned portion of the stream beyond and below the area of impingement of the stream on the plate is split by splitters 9 and 10 to form three output streams, 24, a middlings stream 25 and a tailings stream 26. The tailings are often discarded but may be again furnished to a concentrator if desired. The middlings are usually directed to pass through a concentrator again, while the heavies 24 may, for example, be collected, dried and passed through magnetic or electrostatic separating machines, all as dictated by the type and constitution of the particular ore and the desired end results. The heavies 24 and middlings 25 are collected in any desired type of launders as is conventional in the art, such launders being omitted from the drawing for simplicity. The tailings 26 may be collected or discarded as required.

The lip 3 should be as nearly as possible horizontal from end to end, and the bottom 4 of the sluice should be horizontal from side to side and inclined downwardly from its wide upper end, at the lip, toward the discharge end at outlet 8 at an angle of between 15 and 25 degrees to the horizontal. The minimum angle of inclination at which build-up of ore particles in the sluice does not occur is preferred, and for a rate of flow of 1.5 tons (dry weight) of ore per hour, and for a pulp of 60% by weight of solids entrained in 40% by weight of water, or 60% pulp density, a slope of 19 degrees has proved satisfactory. Greater pulp density normally requires greater slope, and less density, less slope. The angle of inclination is readily adjusted by means of a turnbuckle 27 which supports the sluice from conduit chamber 2. Chamber 2 is conveniently attached to rigid supporting posts 28 which may, if desired comprise leveling means, not shown, to level lip 3 and sluice bottom 4. The upper end of sluice 5 is connected through pivot pins 29 to the upper end of chamber member 2 permitting adjustment of inclination.

Fig. 2 shows the back of fanning plate 12 which has a pivot post 30 attached thereto. Post 30 carries arms 17 and 18 pivotally thereon, and the arms extend to and under the preferably arcuate lower and forward edge 31 of the plate member. A bolt 32 is threaded through each arm in a position such that screwing in the bolt will cause the arm to be urged or forced away from the back of plate 12 and will cause the arm to be locked in position.

Release is accomplished for adjustment of the arm by unscrewing the bolt a few turns.

The plate has welded thereto a small angle member 33 and the upper portion of the angle member is bolted, by bolt 34, to a second angle member 35, having an adjusting slot through which bolt 34 passes. Angle member 35, in turn, is bolted to a generally upright arm 36, vertically slotted for bolt 37, and which is pivotally adjustably connected by bolt 38 to an arm 39 affixed to the outer surface of sluice wall 6.

The universally adjustable mounting arrangement comprising arm 39, angle 35 and angle 33, together with the several bolts, is further seen in the end view of Fig. 3. As seen in Fig. 3, angle member 35 may be adjusted vertically along arm 36, by loosening bolt 37 and moving the bolt along the slot of arm 36. Arm 36 may be pivotally adjusted on bolt 38 and the bolts 37 and 34 afford means to adjust the angle of the plate. After any adjustments, any of bolts 34, 37 and 38 which have been loosened are, of course, tightened to lock the plate in its adjusted position. The plate, accordingly, may be adjusted as to angles of inclination, as well as up and down, back and forth and in and out.

A spring finger 40 is affixed to the inner surface of each of arms 17 and 18 and each is arranged to bear against the back surface of plate 12 with sufficient force to oppose and normally to prevent unintended changes in position of its respective arm. The arms are locked, however, by tightening the appropriate bolt 32 which engages finger 40 and increases the locking force on the arm. The effect of the respective fingers 40 and bolts 32 is also to draw the splitters 9 and 10 respectively rigidly and firmly against the operative face of plate 12.

The whole inner surface of the sluice, including bottom 4 and side walls 6 and 7, is preferably smoothly faced with neoprene or rubber, which is resistant to wear, and the face 11 of fanning plate 12 is preferably covered with a smooth flat sheet of white rubber or neoprene, made white to permit a ready observation of the minerals concentrations in the fan of minerals on the plate and the concentrations in the several split streams as seen against the plate. Changes which occur in the concentrations are easily recognized against the white plate surface 11 and the splitters may be immediately adjusted to compensate.

The plate surface 11 is herein shown as being flat and a flat plate is preferred. Small amounts of concavity or convexity in the whole plate surface or even in parts of the plate surface are not objectionable, however, and for certain purposes it may be found desirable to provide an appreciable curvature. It will be apparent that the arculate shape of the lower forward edge of the plate is convenient for the type of mounting of the splitters herein shown but that the lower edge shape does not in any way affect the concentration or separation function, it being necessary only that the plate surface extend beyond and below the area of impingement to permit the fanning and vanning functions of the plate.

As a specific example of operation of a fanning concentrator of the type herein disclosed, the concentrator was used to concentrate an ore mined from dunes adjacent the seashore approximately fifteen miles south of the city of Bathurst in Gambia, British West Africa, the ore being a comminuted or granular ore comprising approximately 48% by weight of heavy mineral values, primarily ilmenite, zircon and rutile, with minor amounts of garnet, staurolite and other accessory minerals of slightly less specific gravity than the first three mentioned, but slightly greater specific gravity than the balance of 52% quartz sand. In one pass through a concentrator as shown, utilizing two splitters, the dimensions of the concentrator being substantially those heretofore suggested as exemplary, the following tables indicate the results obtained as measured by the percentage dry weight of the desired heavy minerals contained in the concentrates, middlings and tailings, respectively.

*Gambia ore—as mined*

63.0% pulp density

5 Calculated head feed 48.16% heavy minerals  
Feed rate—2.04 tons per hour, dry weight of ore

|                   | dry wt.,<br>percent | Percent<br>Heavy<br>Mineral |
|-------------------|---------------------|-----------------------------|
| 10                |                     |                             |
| Concentrates..... | 39.5                | 85.4                        |
| Middlings.....    | 30.3                | 34.3                        |
| Tailings.....     | 30.2                | 11.6                        |
| Total solids..... | 100.0               |                             |

*Gambia ore—recleaning tailings from above test to produce final tails for rejection*

20 61.0% pulp density

Calculated head feed 8.74% heavy minerals  
Feed rate—1.99 tons per hour, dry basis

|                   | wt., per-<br>cent | Heavy<br>Mineral,<br>Percent |
|-------------------|-------------------|------------------------------|
| 25                |                   |                              |
| Concentrates..... | 23.9              | 24.8                         |
| Middlings.....    | 45.0              | 5.6                          |
| Tailings.....     | 31.1              | 0.98                         |
| Total solids..... | 100.0             |                              |

35 The above results were obtained by taking timed grab samples and as the percentage of heavy minerals in the new feed vary throughout the bulk the percentage of heavy minerals in the resulting products will vary accordingly. For this reason the tailings for the Test No. 1 do not correspond exactly with the feed to Test No. 2 insofar as heavy mineral content is concerned.

40 While the specific embodiment of this solution shown and described herein comprises, as a pre-conditioner of the pulp, a pinched sluice, it is believed that the most effective stratification and separation of the heavy minerals from the sand particles occurs on the plate surface 11. Stratification also occurs within the deep and narrow stream between the outlet orifice 8 and the point or area of impingement of the stream on the plate. Accordingly, this invention may be practised with a pre-conditioning arrangement other than a pinched sluice, and for some applications commercially practical concentrations may be performed even though the pulp issues from a deep and narrow orifice without any appreciable preconditioning or stratification of the stream before it reaches the orifice.

45 55 While only certain preferred embodiments of this invention have been shown and described by way of illustration, many modifications will occur to those skilled in the art and it is, therefore, desired that it be understood that it is intended in the appended claims to cover all such modifications as fall within the true spirit and 60 scope of this invention.

50 What is claimed as new and what it is desired to secure by Letters Patent of the United States is:

55 65 1. In a wet comminuted ore concentrator, sluice means to provide a thin, deep stream of liquid pulp of generally rectangular cross sectional shape issuing in a predetermined direction from said means with a substantial component of velocity in a horizontal direction, said stream being at least partially stratified to carry a lower strata of heavier ore particles and an upper strata of lighter particles, a plate having a flat surface positioned to intersect said stream at an area of said plate surface spaced from said means, said plate surface being disposed at an average angle of less than twenty degrees to the direction of said issuing stream at said 70 75 area, and being oriented to deflect said stream to one

side, said plate surface extending beyond and below said area, and splitter means positioned against said plate surface and extending generally perpendicularly outwardly therefrom through the spread path of said stream beyond and below said area of said stream-intersected surface plate.

2. In a wet gravity type comminuted ore concentrator, a downwardly inclined trough having side walls gradually converging and having end portions defining the sides of a deep narrow outlet for said trough, a white surfaced plate disposed opposite and beyond said outlet and having a portion of its said surface positioned to be impinged by a liquid stream issuing from said outlet, said portion being substantially flat and slanted at a slight angle to the direction of motion of said issuing stream at said portion, whereby said impinging stream fans out against the surface of said plate generally below and beyond said portion, splitter means extending outwardly from the surface of said plate into said fanned out portion of said stream, and means to adjust the position of said splitter means in directions across said fanned out stream.

3. In a wet gravity comminuted ore concentrator, in combination with means to supply a deep and narrow pulp stream into the air with a substantial component of horizontal velocity, a vanning plate having a surface positioned for impingement by said stream and making an acute angle with the side of said stream, as measured in a plane perpendicular to said side and extending in the direction of stream motion at impingement, said angle being sufficiently small to create little turbulence upon impingement, said surface extending below and beyond the area of impingement and being inclined to the vertical in a direction to retain said stream in fanned out shape thereon, and splitters in said fanned out stream and spaced below and beyond said area of impingement.

4. A wet gravity comminuted ore concentrator comprising means to deliver a stream of pulp in a predetermined direction and with a substantial component of horizontal velocity, said stream having a cross-sectional shape which is deep and narrow, a vanning plate having a surface area disposed to be impinged by said stream at a small angle to said stream direction, said plate extending generally below and beyond said area in a direction to cause said stream as redirected by said impingement on said area to fan out over said plate beyond and below said area, and means for dividing for collection desired fractions of said stream, said means including stream splitters disposed in said fanned out stream and adjustable means connecting said splitters to said plate.

5. In combination, a vertical pulp supply conduit comprising a generally triangular chamber of uniform thickness having an inlet opening into the narrow lower end thereof and having a wide upper outlet bordered on one long side by a lip adapted to supply a thin sheet of pulp thereover, a generally triangular trough having a flat downwardly inclined bottom, wide at the top and disposed at the top under and adjacent said lip to receive said sheet of pulp flowing over said lip, said trough having upstanding side walls confining the stream of pulp on said bottom and gradually converging toward the lower end of said trough and forming at said lower end a narrow high outlet opening, a fan plate having a preferably flat front face and a back portion, universally adjustable mounting means connecting said plate at said back portion to an exterior portion of said trough, said means being adapted and arranged to support said plate with said front face thereof in position to be impinged upon by the stream of pulp issuing from said outlet, a mounting arm pivotally attached to said back portion on a pivot axis spaced upwardly of the lower edge of said fan plate, said arm extending to said edge and under said edge, a splitter member attached to said arm and disposed against said front face and adjustable in position on said front face by

swinging of said arm on said pivot axis, and releasable force means engaging between said back portion and said arm operative to urge said arm and back portion apart, thereby to force said splitter member into contact with said front face and releasably to lock said splitter member in its adjusted position.

6. In a pinched sluice comminuted ore concentrator having an outlet orifice for delivering with a substantial horizontal velocity component a deep narrow liquid stream with particles stratified in accord with their relative specific gravities entrained therein, a fanning member having a surface portion disposed in spaced relation to said outlet orifice and in position to be impinged upon by said liquid stream at an average impingement angle as measured between the side of said stream and said surface portion of not more than substantially 25 degrees whereby turbulence of said stream upon impingement is minimized, said surface portion being inclined from the vertical by an angle greater than said average angle, the surface of said plate extending below and beyond said impinged portion thereof and being adapted and arranged to van and fan said stream, and splitter means positioned below and beyond said impinged portion to split said fanned stream into at least two streams having respectively 20 different concentrations of particles of different specific gravities.

7. In a comminuted material concentrator, downwardly inclined preliminary stratification planar surface means, means to deliver a substantially constant flow of said material to the upper end of said surface, means to restrict the material between lateral bounds on said surface, said last means being arranged to constrict and direct said material into a narrow outlet path at the lower end of said surface, the inclination of said surface being sufficient 30 to cause said material to flow thereover under the force of gravity from said upper to said lower end, a fanning plate positioned to intercept the comminuted material in said outlet path following the issuance thereof from said lower end of said surface, said plate being positioned at an acute angle of less than 25 degrees to the direction of motion of said stream at the area of interception thereof and said plate extending downwardly and beyond said area of interception thereby to fan said material over a portion 40 of said plate, and splitter means at said portion disposed to extend outwardly from the surface of said plate.

8. A pinched sluice wet ore concentrator comprising an upstanding generally inverted triangular hollow conduit with a relatively small apical inlet opening at the bottom to receive a flow of ore pulp under pressure and a relatively much larger delivery opening at the top, said delivery opening having a length at least approximately five times its width and having a horizontal delivery lip along a long side thereof, a downwardly inclined trough having a bottom positioned with its upper end parallel to, below 50 and immediately adjacent to said lip and having side walls converging from the upper to the lower end to form an outlet orifice, and splitter means for the stream issuing from said orifice.

9. In a wet comminuted ore concentrator, an upstanding generally inverted triangular hollow conduit with a relatively small apical inlet opening at the bottom to receive a flow of ore pulp under pressure and a relatively much larger delivery opening at the top, said delivery opening having a length at least approximately five times 60 its width and having a horizontal delivery lip along a long side thereof, and stratifying sluice means having an upper end disposed under said lip to receive the ore pulp flowing thereover.

10. The method of separating comminuted ore particles 70 of differing respective specific gravities which comprises the steps of forming a pulp comprising a liquid with said comminuted ore particles suspended therein, flowing said pulp down a flat downwardly inclined surface, gradually increasing the stream width of said pulp along its direction of flow on said surface, permitting said re-

stricted width stream to issue freely over a lower edge of said surface, intercepting said freely flowing pulp stream with a planar surface so positioned and canted as to locate the area of impingement of said stream thereon spacedly beyond and below said lower edge and as to form an angle of interception of said stream of less than 25 degrees, and splitting the stream fanned on said planar surface.

11. The method of concentrating comminuted ore and the like wherein a deep and narrow stream of ore or the like pulp with a substantial component of horizontal velocity is directed against a vanning plate which extends at a sufficiently acute angle to the direction of the stream just prior to impingement, as measured in a horizontal plane, to create little turbulence on impingement and which extends below and beyond the area of impingement, and said fanned out stream is split into a plurality of separate streams.

12. In an ore concentrator, a plate having an arcuate edge, means to impinge moving ore particles against a front surface of said plate to fan toward said arcuate edge, a splitter member having a splitting edge directed into the fanned path of said particles and having an end of said member in contact with said surface, a pivot on the back of said plate equidistant from spaced points of said arcuate edge, an arm structure supported on said pivot and extending to and around said edge and having a swingable end affixed to said splitter member, said arm

structure comprising force means engageable with the back of said plate urging said arm structure away from said back surface thereby to urge said splitter member toward said front surface.

- 5 13. In an ore concentrator, a plate having an arcuate edge, means to impinge ore particles against a front surface of said plate to fan toward said arcuate edge, a splitter member having a splitting edge directed into the fanned path of said particles and having an end of said member in contact with said surface, a pivot on the back of said plate equidistant from spaced points of said arcuate edge, an arm structure supported on said pivot and extending to and around said edge and having a swingable end affixed to said splitter member, said arm structure  
10 15 comprising force means engageable with the back of said plate urging said arm structure away from said back surface thereby to urge said splitter member toward said front surface, said force means comprising manually operable means for adjusting the amount of urging force on  
20 said arm structure.

**References Cited in the file of this patent**

**UNITED STATES PATENTS**

|    |           |            |               |
|----|-----------|------------|---------------|
| 25 | 977,956   | Langerfeld | Dec. 6, 1910  |
|    | 1,828,760 | Blatch     | Oct. 27, 1931 |
|    | 2,644,583 | Cannon     | July 7, 1953  |